

## UNITED STATES PATENT OFFICE

2,213,397

## ALLOYS

Edwin F. Kingsbury, Rutherford, and Howard T. Reeve, Millburn, N. J., assignors to Bell Telephone Laboratories, Incorporated, New York, N. Y., a corporation of New York

No Drawing. Original application July 10, 1937, Serial No. 152,993. Divided and this application October 18, 1938, Serial No. 235,560

8 Claims. (Cl. 148—11.5)

This is a divisional application of U. S. Patent 2,148,562, Serial No. 152,993 filed July 10, 1937 granted to E. F. Kingsbury and H. T. Reeve on February 28, 1939.

5 This invention relates to contacting alloys and more particularly to copper-palladium alloys employed for contacts on electrical apparatus. An object of this invention is to increase the efficiency and prolong the usefulness of contacts 10 employed on electrical apparatus.

The contacts of electrical apparatus, especially relay contacts, are subjected to severe conditions in use. The minute sparking in the operation of the contacts of relays and other apparatus 15 causes the building-up of the material on the contacts to render ultimately the relay inoperative. Various materials which withstand these severe conditions have been suggested. For example, E. F. Kingsbury in U. S. Patent 1,779,602 20 granted on October 28, 1930, has proposed the use of copper-palladium and other alloys for electrical contacts. The alloys of palladium-copper while possessing relative freedom from excessive oxidation and in general satisfactory as 25 a contacting material are somewhat susceptible, as ordinarily prepared, to the building-up phenomena in which material is transferred from one contact to another.

The major factors which are correlated with 30 the transferring of the material of one contact to that of another are the thermal and electric conductivity of the alloy. An alloy having a higher thermal and electric conductivity than that of another alloy comprising the same constituents is less prone to the transferring and 35 building-up in needle-like fashion of the material of one contact on that of another.

In accordance with this invention copper-palladium alloys are prepared which have relatively high thermal and electrical conductivities 40 and which are resistant to corrosion such as that caused by sulphur dioxide. Further, these alloys when employed for contacts on relays and other electrical apparatus manifest greater resistance 45 to the transfer of metal from one contact to another.

Copper-palladium alloys, and more particularly 50 alloys comprising 38 to 50 atomic per cent of palladium and the remainder chiefly copper exist in two extreme physical conditions, one, in which the atoms of the two elements are distributed at random, and the other in which the distribution is ordered. In the ordered condition, the two elements are in preferred positions with respect 55 to each other, or more concretely, the elements

are positioned so that an atom of one element is nearer the atom of the other element. The lattice structure of the ordered state is the body centered cube, while the lattice structure of the random state is the face centered cube. The 5 copper-palladium alloys as usually prepared are in a random state, or in any case, are only partially ordered. Certain characteristics of copper - palladium alloys undergo profound changes when converted from the random to the 10 ordered state. The electrical resistivity of an alloy comprising 47.2 atomic per cent palladium and 52.8 atomic per cent copper (60 per cent palladium and 40 per cent copper by weight) in the ordered condition is less than approximately 15 one-tenth of that in its random state. The specific resistivity of the ordered alloy comprising 47.2 atomic per cent palladium and 52.8 atomic per cent copper is less than  $4 \times 10^{-6}$  ohm-cm. This resistivity is considerably less than that of 20 palladium itself in spite of the fact that the alloy is almost in the center of the binary series. The ordered alloys are substantially harder than the corresponding alloys in the random state and the thermal conductivity is substantially greater 25 in the ordered alloys. This greater hardness is of value when contacts are subjected to constant battering action such as that which obtains in high speed telegraph relays. The ordered structure of the alloys also has been found to result 30 in decreased chemical corrosion on exposure to hydrogen sulphide and sulphur dioxide. The decreased resistivity, the increased thermal conductivity, hardness and resistance to corrosion contribute to make alloys of copper-palladium in 35 the ordered state extremely desirable as contact alloys for relays and other electrical apparatus.

One method of preparing the copper-palladium alloy in the ordered state is to cold work the 40 alloy and subsequently heat treat it within a temperature range of 275° C. to 450° C. The cold working may be effected by reducing the cross-sectional area of the alloy in the order of less than 50 per cent of that of the original. For example, an alloy comprising 50 per cent atomically of palladium and 50 atomic per cent of copper (62.7 per cent palladium and 37.3 per cent copper by weight) in the form of a wire .050 inch in diameter, is reduced to a diameter of .005 inch. This wire is then wound on a form, leads 50 are welded on the wire for the determination of the resistance thereof and the form placed in a quartz tube which is maintained at a temperature of 280° C. This heat treatment may be performed in vacuum or in the presence of an 55

inert gas which does not react with the copper-palladium alloy. The resistivity of the wire is determined from time to time in order to ascertain whether the transformation from the 5 random state to the ordered state has been effected. A period of 15 to 30 minutes has been found satisfactory for this size of wire. Usually, the greater the degree of hard working prior to heating, the lesser time is required for the transformation. In any event the alloy is left in the furnace until the transformation is effected. As ascertained by resistance measurements, the specific resistivity for this particular alloy in the ordered state is  $4.1 \times 10^{-6}$  ohm-cm. After the 10 transformation has been accomplished, the wire in the furnace is permitted to cool slowly therein to room temperature. With a wire .005 inch in diameter, the transformation from the random to the ordered state occurs in less than seven 15 minutes at a temperature range of 290° C. to 330° C. Although the transformation is produced in this period, the alloy is preferably subjected to the heating for a longer time, such as 15 to 30 minutes. The transformation may also be 20 ascertained by X-ray examination although the resistivity determination is more convenient.

While two specific alloys of copper-palladium have been noted, any other alloy of copper-palladium, consisting of 38 to 50 per cent atomically 30 of palladium (50.7 to 62.7 per cent palladium by weight) and the remainder chiefly copper, may be treated in like manner to change them from the random to the ordered state. The period of heating in each case is relatively short and 35 can be easily ascertained by resistivity measurements.

While preferred embodiments of this invention have been described, various modifications therein may be made without departing from the scope 40 of the appended claims.

What is claimed is:

1. The method of forming an improved contact alloy consisting of 50.7 to 62.7 per cent palladium by weight and 49.3 to 37.3 per cent copper by weight, said method comprising cold working said alloy and heat treating said alloy at a temperature of 275° C. to 450° C. to change the atomic relation of said palladium and said copper from a random to an ordered state.

2. The method of forming an improved contact material consisting of 50.7 to 62.7 per cent palladium by weight and 49.3 to 37.3 per cent copper by weight, said method comprising cold working said alloy by reducing the cross-sectional area thereof, heating said alloy to a temperature of

approximately 280° C. to effect the transformation of said copper and said palladium from a random to an ordered state and slowly cooling said alloy to room temperature.

3. A contact material consisting of 50.7 to 62.7 per cent palladium by weight and 49.3 to 37.3 per cent copper by weight, said alloy being prepared by cold working and subsequent heat treatment at a temperature between 275° C. to 450° C. to convert said palladium and said copper from a random to an ordered state. 5

4. A contact material consisting of approximately 60 per cent palladium by weight and approximately 40 per cent copper by weight, said alloy being prepared by cold working and subsequent heat treatment at a temperature between 275° C. to 450° C. to convert said palladium and said copper from a random to an ordered state. 15

5. A contact material consisting of approximately 62.7 per cent palladium by weight and 37.3 per cent copper by weight, said alloy being prepared by cold working and subsequent heat treatment at a temperature between 275° to 450° C. to convert said palladium and said copper from a random to an ordered state. 20

6. The method of forming an improved contact alloy consisting of 50.7 to 62.7 per cent palladium by weight and 49.3 to 37.3 per cent copper by weight, said method comprising cold working 30 said alloy by reducing the cross-sectional area thereof to the order of less than 50 per cent of that of the original and heat treating said alloy at a temperature between 275° C. and 450° C. to change the atomic relation of said palladium and 35 said copper from a random to an ordered state.

7. The method of forming an improved contact alloy consisting of 50.7 to 62.7 per cent palladium by weight and 49.3 to 37.3 per cent copper by weight, said method comprising cold working 40 said alloy, heating said alloy to a temperature at which it is converted from a random to an ordered state, maintaining said alloy at said temperature for a time sufficient to cause conversion to the ordered state and cooling said alloy. 45

8. A contact element consisting of 50.7 to 62.7 per cent palladium by weight and 49.3 to 37.3 per cent copper by weight, said alloy being prepared by cold working, subsequent heating to a temperature at which said alloy is converted from a 50 random to an ordered state for a time sufficient to cause conversion to the ordered state, and subsequent cooling.

EDWIN F. KINGSBURY.  
HOWARD T. REEVE.

55